

Nov. 10, 1953

G. GUTZEIT ET AL

2,658,841

PROCESS OF CHEMICAL NICKEL PLATING AND BATH THEREFOR

Filed Nov. 8, 1950

7 Sheets-Sheet 1



FIG. I

INVENTORS  
Gregoire Gutzeit  
BY Abraham Krieg  
Smith, Olm & Baird,  
Attns.

Nov. 10, 1953

G. GUTZEIT ET AL

2,658,841

PROCESS OF CHEMICAL NICKEL PLATING AND BATH THEREFOR

Filed Nov. 8, 1950

7 Sheets-Sheet 2



FIG. 2



FIG. 3

INVENTORS  
Gregoire Gutzeit  
Abraham Krieg  
Smith, Alen & Baird,  
Attns.

BY

Nov. 10, 1953

G. GUTZEIT ET AL

2,658,841

PROCESS OF CHEMICAL NICKEL PLATING AND BATH THEREFOR

Filed Nov. 8, 1950

7 Sheets-Sheet 3



FIG. 4



FIG. 5

BY

Smith, Olsen & Baird,  
Attys.

Nov. 10, 1953

G. GUTZEIT ET AL

2,658,841

PROCESS OF CHEMICAL NICKEL PLATING AND BATH THEREFOR

Filed Nov. 8, 1950

7 Sheets-Sheet 4



FIG. 6



FIG. 7

INVENTORS

Gregoire Gutzeit  
Abraham Krieg

Smith, Olaw & Baird,  
Atty's.

Nov. 10, 1953

G. GUTZEIT ET AL

2,658,841

PROCESS OF CHEMICAL NICKEL PLATING AND BATH THEREFOR

Filed Nov. 8, 1950

7 Sheets-Sheet 5



FIG. 8



FIG. 9

INVENTORS  
Gregoire Gutzeit  
BY Abraham Krieg  
Smith, Alen & Baird,  
Atty.

Nov. 10, 1953

G. GUTZEIT ET AL

2,658,841

PROCESS OF CHEMICAL NICKEL PLATING AND BATH THEREFOR

Filed Nov. 8, 1950

7 Sheets-Sheet 6



FIG. 10



FIG. 13

INVENTORS  
Gregoire Gutzeit  
BY      Abraham Krieg  
Smith, Olser & Baird,  
Atty's.

Nov. 10, 1953

G. GUTZEIT ET AL

2,658,841

PROCESS OF CHEMICAL NICKEL PLATING AND BATH THEREFOR

Filed Nov. 8, 1950

7 Sheets-Sheet 7



INVENTORS

Gregoire Gutzeit

BY Abraham Krieg

*Smith, Olsen & Baird,*  
Atty's.

## UNITED STATES PATENT OFFICE

2,658,841

PROCESS OF CHEMICAL NICKEL PLATING  
AND BATH THEREFOR

Gregoire Gutzeit, Highland, and Abraham Krieg,  
Gary, Ind., assignors to General American  
Transportation Corporation, Chicago, Ill., a cor-  
poration of New York

Application November 8, 1950, Serial No. 194,656

12 Claims. (Cl. 117—130)

1

The present invention relates to processes of chemical nickel plating and to baths employed in carrying out such processes.

The purpose of the invention is to provide a chemical plating process which will have many advantages in commercial use over electroplating methods, including low cost of equipment, good adhesion of the coating in the finished product, high corrosion resistance of the coating, and a coating which is uniform, continuous and much harder.

Efforts have heretofore been made to obtain some of these desirable results by coating processes but without sufficient success to warrant the commercial use of the methods suggested. For example, it has been proposed by Brenner and Riddell (Jour. Research, National Bureau of Standards, vol. 37, July, 1946, and vol. 39, November, 1947) that coatings of nickel may be deposited upon the surfaces of catalytic metals, for example, mild steel, by employing a chemical reduction of nickel ions from an aqueous bath containing hypophosphite ions in the presence of sodium ions and sulfate ions and using sodium acetate as a buffer to maintain the pH of the bath in the range of from 4 to 6, the temperature of the bath being maintained at about 90° centigrade. For instance, Brenner and Riddell suggest a number of baths one of which comprises nickel sulfate (30 gms./liter), sodium hypophosphite (10 gms./liter), and sodium acetate (10 gms./liter). In all of these baths, the ratio of nickel ions to hypophosphite ions



expressed in terms of molar concentrations as a decimal fraction, is approximately 1.33, and the absolute concentration of hypophosphite ions is approximately 0.095 mole/liter. Employing this bath Brenner and Riddell obtained the deposition of the nickel upon the surface of the steel at a rate of 0.015 millimeter per hour.

In such a chemical plating process, the principal reaction, in the presence of water, expressed in ionic form is considered to be:



For instance, using nickel chloride to provide the nickel ion and sodium hypophosphite to provide the hypophosphite ion:



While the process of Brenner and Riddell offers certain advantages over competitive electrolytic

processes, it was found by them to be uneconomical, to produce deposits at a slow rate and to lack control of the composition of the deposits. It is considerably more expensive to carry out than the competing electrolytic processes due primarily to the low nickel efficiency of the reaction, i. e., the per cent of nickel actually deposited at completion, as related to the total amount of nickel present in the bath initially.

10 Accordingly, it is a general object of the present invention to provide an improved chemical nickel plating process of the general character described, in which the reaction involved is carried out in an efficient manner which renders the process economical from a commercial and industrial standpoint.

Another object of the invention is to provide an improved aqueous bath of the general character described that may be employed with advantage in carrying out the improved process.

A further object of the invention is to provide an improved process of chemical nickel plating and an improved aqueous bath that may be employed in carrying out the process, whereby the surfaces of catalytic materials may be readily coated with nickel in a simple and efficient manner and wherein the nickel coatings are smooth and continuous and are of a low porosity and of high corrosion resistance and are intimately bonded to the surface of the catalytic material.

35 A further object of the invention is to provide an improved process of chemical nickel plating and an improved aqueous bath that may be employed in carrying out the process that are adapted for the commercial coating of iron, steel and the like.

Further features of the invention pertain to the particular arrangement of the steps of the process and to the composition of the aqueous bath, whereby the above mentioned objects of the invention and others are attained.

The invention, both as to its organization and principle of operation, together with further objects and advantages thereof, will best be understood by reference to the following specification taken in connection with the accompanying drawings, in which,

50 Figure 1 shows the relative amounts of plating deposited with changes in temperature;

Fig. 2 shows the variation of the weight of plating deposited in a given period with variation of the ratio of nickel ions to hypophosphite ions;

Fig. 3 shows the change in the pH value after a given period with variation of the ratio of nickel ions to hypophosphite ions;

Fig. 4 shows the variation in the weight of the

plating deposited in a given time with variation in the hypophosphite ion concentration;

Fig. 5 shows the weight of the plating deposited in a given period with variation in the ratio of nickel ions to hypophosphite ions when using the hypophosphite ion concentration employed by Brenner and Riddell as compared with the use of the higher concentration involved in the discovery of the present invention;

Fig. 6 shows the variation of the weight of the plating deposited with variation in the ratio of nickel ions to hypophosphite ions when using a higher ratio of bath volume to plating surface area than that employed in the tests recorded by the curves of Fig. 5;

Fig. 7 shows the variation of the weight of the plating deposited with variation in the ratio of nickel ions to hypophosphite ions derived from sodium hypophosphite;

Fig. 8 shows the variation in nickel efficiency, in per cent at completion, with variation in the ratio of nickel ions to hypophosphite ions;

Fig. 9 shows a series of curves illustrating the variation in the weight of the plating deposit with variation in the pH of the plating bath for different specified ratios of nickel ions to hypophosphite ions derived from sodium hypophosphite;

Fig. 10 shows the variation in weight of the plating deposit with variation in the ratio of nickel ions to hypophosphite ions derived from sodium hypophosphite for two specified pH values for the bath;

Figs. 11 and 12 show a series of curves illustrating the variation in the weight of the plating deposit with variation in the pH of the plating bath for different ratios of nickel ions to hypophosphite ions derived from calcium hypophosphite; and

Fig. 13 shows the variation of the weight of the nickel plating deposit with variation in the ratio of nickel ions to hypophosphite ions derived from calcium hypophosphite with the use of calcium acetate as a buffer.

In accordance with the process of the present invention, the catalytic material that may be coated with nickel comprises any material in the solid phase which will initiate at its surface the reaction of Equations 1 and 2 set forth above; i. e., a material which, when immersed in the bath, will cause the evolution of hydrogen gas at its own surface. The following elements are examples of catalytic materials which may be nickel plated: copper, silver, gold, beryllium, boron, germanium, aluminum, thallium, silicon, carbon, vanadium, molybdenum, tungsten, chromium, selenium, tellurium, titanium, iron, cobalt, nickel, palladium and platinum; and the following elements are examples of noncatalytic materials which ordinarily may not be nickel plated: bismuth, cadmium, tin, lead and manganese. The activity of these catalytic materials varies considerably. The following elements are particularly good catalysts in the chemical nickel plating bath hereinafter set forth, viz: aluminum, carbon, chromium, cobalt, iron, nickel and palladium.

Thus, the nickel plating process becomes autocatalytic, when both the original surface and the metal that is deposited are catalytic, and the reduction of the nickel salt to metallic nickel in the bath in accordance with the reaction of Equation 2 proceeds until all of the nickel ions have been reduced to metallic nickel, in the presence of an excess of hypophosphite ions, or until

all of the hypophosphite ions have been oxidized to phosphite, in the presence of an excess of nickel ions. Actually the reaction of Equations 1 and 2 is slowed down rather rapidly as time elapses, because the anions, as contrasted with the cations, of the nickel salt combine with the hydrogen cations to form an acid, which, in turn, lowers the pH of the bath tending to dissolve the nickel deposit. This reaction is considered to be:



Also, the reducing power of the hypophosphite ion is decreased as the pH value decreases. It is, therefore, important to prevent a rapid drop of the pH of the bath after initial adjustment thereof within its optimum range. This can be achieved by various schemes both alone and in combination. For example, a soluble nickel salt of a weak acid, such as acetic acid, can be used both to provide nickel ions and to act as a buffer. Also, the pH of the bath can be corrected periodically by the addition of a weak alkali, such as sodium bicarbonate; or a buffer, such as sodium acetate or other alkali acetate, can be added to the bath.

In carrying out the process, the article to be plated and normally formed of the catalytic material is properly prepared by mechanically cleaning, degreasing and light pickling, according to the standard practice in electroplating processes. For example, in the nickel plating of a steel object, it is customary mechanically to clean the rust and mill scale from the object, to degrease the object, and then lightly to pickle the object in a suitable acid, such as HCl. The article is then immersed in a suitable volume of the aqueous bath containing the proper proportions of nickel ions, hypophosphite ions and a buffer, the pH of the bath having been first adjusted to an optimum value by the addition of a suitable acid, and the bath having been heated to a temperature just below its boiling point, such as 99° C. at atmospheric pressure. Almost immediately, hydrogen bubbles can be observed forming on the catalytic surface of the steel object and escaping in a steady stream from the bath, while the surface of the steel object is slowly coated with nickel (containing some phosphorus). The reaction is continued until the color of the bath (green at the start) shows the absence of nickel, or until the evolution of hydrogen gas stops.

A nickel plating bath, as indicated above, containing a soluble nickel salt, a soluble hypophosphite and a buffer, is only relatively stable; and even without the presence therein of a catalytic surface, it tends to decompose more or less rapidly by random chemical reduction of the nickel ions. Specifically, the nickel ions are reduced as a fine amorphous, black powder, which, in turn, acts as a catalyst. The resulting precipitate is gray to black and contains various quantities of nickel, phosphorus and salts, depending on the conditions of formation. This spontaneous decomposition is a function of temperature, time and initial bath composition; and insofar as the initial bath composition is concerned, the higher the ratio of hypophosphite ions to nickel ions and the higher the absolute concentration of hypophosphite ions, the more unstable is the bath. In other words, instead of a bath capable of controlled nickel deposition in the presence of a catalyst, a high concentration of hypophosphite anions will produce the well-known purely chemical nonselective reduction of nickel ions. Under plating conditions, in the presence of a catalytic

surface and at an elevated temperature, the tendency to form this black precipitate is even more pronounced. The formation of the black precipitate in the bath is highly objectionable in that the presence of the conditions causing the black precipitate in the bath result in a rapid decomposition of the bath by the uncontrolled chemical reduction of the nickel ions in the bath, thus depleting the bath. Also, the presence of the black precipitate in the bath results in a dull, rough and uneven nickel coating upon the object that is undergoing the plating reaction.

In carrying out the process, the rate of catalytic reduction of nickel ions to metallic nickel is a function of temperature of the bath and this function is logarithmic; for example, if the temperature of the bath is decreased from approximately 100° C. to approximately 90° C., it has been discovered that the plating rate drops approximately 52.5%. It is, therefore, important that the temperature of the bath be maintained at the highest possible temperature below the boiling point thereof under the prevailing conditions, which is under standard conditions a temperature of approximately 99° C. Tests have been made to determine the weight of nickel deposited per hour by the method of the present invention at different temperatures and the results between 90° and 100° C. have been plotted to form the curve 18 shown in Fig. 1 of the drawings.

While it is apparent that there is a definite relationship involving the plating rate of the object in the bath between the volume of the bath and the surface area of the object, it has been discovered that the volume of the bath also determines the relative amount of black precipitate that is formed under otherwise similar conditions. Thus, as the volume increases, the amount of black precipitate increases. Employing the notation "V/A" for the ratio between the volume of the bath expressed in cubic centimeters ( $\text{cm}^3$ ) and the geometric surface area of the object being plated, expressed in square centimeters ( $\text{cm}^2$ ), it has been found that the best values are below 10.

Turning now to the composition of the bath, it essentially comprises an aqueous solution containing nickel ions and hypophosphite ions and a buffer and may be suitably formed employing a soluble nickel salt, a soluble hypophosphite and an acetate. For example, the nickel ions may be derived from nickel chloride or nickel acetate, and the hypophosphite ions may be derived from sodium, potassium, lithium, calcium, magnesium, strontium, barium, etc., hypophosphites or various combinations thereof. It has been found that certain alkaline cations that are thus introduced into the bath appear to retard the rate of nickel deposition with respect to other cations. For example, barium ions appear to retard the rate of nickel deposition with respect to sodium and potassium ions. On the other hand, certain cations that are thus introduced into the bath appear to accelerate the rate of nickel deposition with respect to other cations. For example, magnesium ions appear to accelerate the rate of nickel deposition with respect to sodium and potassium ions. Accordingly, from a standpoint of economy, sodium and calcium hypophosphites are recommended; and from a standpoint of realizing the maximum rate of nickel deposition, magnesium hypophosphite is recommended.

In preparing the bath, the amounts of soluble nickel salt and soluble hypophosphite that are employed are such that both the ratio of nickel ions to hypophosphite ions and the absolute concentration of hypophosphite ions are initially established within optimum ranges. The term "ion" as employed herein includes the total quantity of element or radical present in the bath; i. e., both undissociated and dissociated material. In other words, 100% dissociation is assumed when the term "ion" is used in connection with molar ratios and concentrations in the bath. The ratio between the nickel ions and the hypophosphite ions,  $\text{Ni}^{++}/(\text{H}_2\text{PO}_2)^-$ , in terms of molar concentration may be expressed as a decimal fraction; and it has been discovered that the most favorable range of this fraction lies between 0.25 and 0.60. It has also been discovered that the required absolute concentration of the buffer anions, such as acetate ions, should be equivalent to two carboxyl groups per ion of nickel that can be reduced, as explained more fully hereinafter. For example, if a hypophosphite ion concentration of .225 mole/liter is chosen, the required absolute concentration of acetate ions of the buffer, expressed in mole/liter, would be approximately 0.120.

The relationship between the ratio,



and nickel plating rates is illustrated by the curve 29 of Fig. 2 of the accompanying drawings. This curve has been plotted with the results of a test in which the object plated was formed of mild steel, the absolute concentration of hypophosphite ions was 0.095 mole/liter, as in the Brenner and Riddell baths, derived from sodium hypophosphite, the absolute concentration of acetate ions was 0.120 mole/liter, the V/A ratio was 100/5, the temperature of the bath was approximately 99° C., and the initial pH of the bath was in the range of from 5.38 to 5.49. In Fig. 2 the abscissae show the ratio of nickel ions to hypophosphite ions and the ordinates show the weight of the plating deposited in a period of two hours in milligrams per square centimeter. It will be observed that the highest plating rates were obtained when the ratio of nickel ions to hypophosphite ions was in the range 0.25 to 0.60. In the zone where the highest plating rate was obtained, the coating was also of the best quality, being bright and smooth. The lower plating rates were characterized by a dull and rough coating. The zone where the coating was bright and smooth has been indicated in Fig. 2 by the notation *bs* and the zone where the coating was dull and rough has been indicated by the notation *dr*.

In the event the absolute concentration of hypophosphite ions in the bath is increased while maintaining constant the nickel ions to hypophosphite ions ratio, an increased rate of nickel deposition is realized, until a region is reached where the bath becomes unstable such that spontaneous decomposition thereof takes place with the resulting formation of the black precipitate previously referred to.

It has been discovered that the optimum absolute concentration of hypophosphite ions in the bath, i. e., one that will result in good nickel plating without an excessive tendency to spontaneous decomposition, is within the range 0.15 mole/liter to 0.35 mole/liter; and approximately 0.225 mole/liter is recommended. Moreover, the spontaneous decomposition of the bath with a constant absolute concentration of hypophosphite

ions is related to the ratio,  $\text{Ni}^{++}/(\text{H}_2\text{PO}_2)^-$ , as illustrated by the curve 22 shown in Fig. 3 which shows, with varying ratios of nickel ions to hypophosphite ions, the drop in pH value after three hours at 99° C. without a catalyst.

In these tests, represented by the curve 22 of Fig. 3, the absolute concentration of hypophosphite ions was 0.224 mole/liter; the absolute concentration of acetate ions was 0.120 mole/liter; the temperature of the bath was approximately 99° C.; and the initial pH of the bath was in the range 4.90 to 5.01. From Fig. 3, it will be observed that the minimum spontaneous decomposition, as determined by the drop in pH of the bath after three hours, occurred when the ratio



was in the range 0.25 to 0.60. Of course, it will be appreciated that the pH drop of the bath is a direct function of the spontaneous decomposition thereof, since the uncontrolled chemical reduction of the nickel cation will produce the acid corresponding to the anion of the originally employed nickel salt in amounts corresponding to its mass. In these tests, as well as in the others herein referred to, the pH values were determined at room temperature.

It will be understood that the higher absolute hypophosphite ion concentrations yield higher rates of deposition of the nickel without materially impairing the stability of the bath within the optimum  $\text{Ni}^{++}/(\text{H}_2\text{PO}_2)^-$  ratio. On the other hand, if the absolute concentration of hypophosphite ions is increased substantially above the optimum range (0.15 mole/liter to 0.35 mole/liter), both the amount of nickel plating obtained during a given period and the quality of coating are considerably decreased by virtue of the random chemical reduction of the nickel ions that takes place and produces the black precipitate which, in turn, causes roughness and porosity in the coating, as previously mentioned. This circumstance is illustrated by the curve 24 of Fig. 4 which shows as abscissae the concentration of the bath and, as ordinates, the weight of the plating deposited in periods of two hours, in milligrams per square centimeter.

In these tests, the results of which are plotted in Fig. 4, the object plated was formed of mild steel; the  $\text{Ni}^{++}/(\text{H}_2\text{PO}_2)^-$  ratio was 0.330; the V/A ratio was 100  $\text{cm}^3/5 \text{ cm}^2$ ; the temperature of the bath was approximately 99° C.; and the initial pH of the bath was approximately 5.0. These tests showed a maximum plating deposit with a hypophosphite concentration of 0.224 and this coating was bright and smooth with only a trace of black precipitate but as the concentration increased the black precipitate increased very rapidly and the plating became very rough. As the hypophosphite ion concentration is decreased below the preferred value, the black precipitate is only a trace and the plating is good but dull in appearance.

For purposes of comparison and to demonstrate the advantages of the discoveries of the present invention, tests have been made using sodium hypophosphite and an absolute concentration of hypophosphite ion equal to that specified by Brenner and Riddell for their bath No. 4 (and in the same order of magnitude as in their other baths), viz., 0.095 moles per liter, in coating a mild steel sample with a fixed acetate concentration of .120 mole/liter, at a V/A ratio of 50  $\text{cm}^3/20 \text{ cm}^2=2.5$ , at an initial pH of about 5.5 and at a bath temperature of 99° C. for a period of thirty minutes, with the results which

are shown by curve 26 in Fig. 5, where the abscissae show the ratio of nickel ions to hypophosphite ions and the ordinates show the weight of the plating deposited in milligrams per square centimeter. With this low nickel hypophosphite ion concentration, it was found that when the ratio of nickel ions was very low (between .179 and .368) there was no plating deposit. The plating was at a maximum when the ion ratio was .368 and it gradually decreased as this ratio increased. The plating was good until the ratio of 1.325 was reached when it appeared slightly stained.

Using the same baths with sodium hypophosphite, these tests were repeated at a V/A ratio of 2.5 and at a temperature of 99° C. with the hypophosphite ion concentration constant at .224 mole/liter and the results are shown by the curve 28 in Fig. 5. Thus by substantially doubling the absolute hypophosphite ion concentration used by Brenner and Riddell, considerably higher rates of deposition can be obtained, while the stability of the baths is very little impaired at the optimum  $\text{Ni}^{++}/(\text{H}_2\text{PO}_2)^-$  ratio. When the ratio of nickel ions to hypophosphite ions was in the range between 0.2 and 0.6, the nickel plating was good and very bright.

With the same absolute concentration of hypophosphite ion (.224 mole/liter) derived from sodium hypophosphite as in the tests represented by curve 28 in Fig. 5, and using a similar series of baths, but plating at a higher V/A ratio ( $50 \text{ cm}^3/5 \text{ cm}^2=10$ , at a temperature of about 99° C., the amount of nickel deposited in 60 minutes, with an initial pH of 5.50, was as shown by the curve 30 in Fig. 6. At the lower ratios of nickel ions to hypophosphite ions the weight of the plating deposit was substantially greater and it was brightest and smoothest in the region represented by the peak of the curve.

On further tests, using again the same absolute concentration of hypophosphite ion (.224 mole/liter) derived from sodium hypophosphite and with the same baths, but plating at a still higher V/A ratio ( $100 \text{ cm}^3/5 \text{ cm}^2$ ) at about 99° C. the amount of nickel deposited in two hours was as indicated by the curve 32 in Fig. 7. The deposit was dark and nonmetallic under the conditions represented by the beginning of the curve but was good at all other times. A study of the curves shown in Figs. 2, 5, 6 and 7 shows a definite maximum weight of deposit when the ratio  $\text{Ni}^{++}/(\text{H}_2\text{PO}_2)^-$  is between 0.25 and 0.6.

So far as nickel efficiency is concerned, i. e., the weight of available nickel deposited (including the nickel-phosphorus compound), it decreases as the ratio  $\text{Ni}^{++}/(\text{H}_2\text{PO}_2)^-$  increases as is shown by the curve 34 in Fig. 8, using the same bath as that employed for the experiments represented by the curve 26 in Fig. 5, and with a hypophosphite concentration of 0.095 mole/liter. The region of optimum ratio (between 0.25 and 0.60) proved vastly superior to that used by Brenner and Riddell. With an absolute hypophosphite ion concentration of .224 mole/liter the nickel efficiency at completion was 97.5% for a  $\text{Ni}^{++}/(\text{H}_2\text{PO}_2)_2$  ratio of .357 and 25.0% for a  $\text{Ni}^{++}/(\text{H}_2\text{PO}_2)_2$  ratio of 1.33 (B. & R.).

As previously indicated, a low pH in the bath will increase the pressure of dissolution of the catalyst (if the catalyst is acid soluble) and of the deposited nickel according to the Reaction 3 appearing above and will lower the reducing power of the hypophosphite. On the other hand, a high pH tends to favor the formation and eventual precipitation of basic nickel salts and to pro-

9  
mote "crusting" at the catalytic surface. As shown above, the optimum plating results with a simple bath containing nickel ions, hypophosphite ions and acetate ions, can be obtained by using a hypophosphite ion concentration of around 0.2 mole/liter and a  $\text{Ni}^{++}/(\text{H}_2\text{PO}_2^-)$  ratio of about 0.25 to 0.60. Plating solutions were prepared, according to these teachings, containing 0.224 mole/liter of hypophosphite ion derived from sodium hypophosphite with variable  $\text{Ni}^{++}/(\text{H}_2\text{PO}_2^-)$  ratios and the usual buffer concentration (0.120 mole/liter). The initial pH was adjusted by the addition of acetic acid. Using a medium V/A ratio of 50  $\text{cm}^3$  volume on 5  $\text{cm}^2$  area of catalyst (iron), the deposits of nickel in 60 minutes at 99° C. were as shown by the curves 35, 38 and 40 in Fig. 9.

It will be observed that Fig. 9 shows two optimum initial pH values when sodium hypophosphite is used and when the maximum amount of nickel deposited is regarded as the only criterion; the first one is at pH 4.60 and the second at pH 5.50. The first appears to yield a higher rate of deposit at the optimum nickel to hypophosphite ratio (0.447 in this series). The average results of a series of tests with two different pH values of 4.6 and 5.6 with respect to weight of nickel deposited with varying ratios of nickel ions to hypophosphite ions, derived from sodium hypophosphite, have been plotted to form the curves 42 and 44, respectively, shown in Fig. 10. With the ratios of nickel ions to hypophosphite ions represented by the peaks of these curves, where the nickel plating deposit was greatest, the plating was also the brightest and smoothest. In general, the lower pH value appeared to give better results both as to the amount of the plating deposit and its brightness.

The results of tests which have been plotted to form the various curves shown in Figs. 1 to 10, inclusive, were made with sodium hypophosphite. For purposes of comparison, reference will now be made to tests which resulted from the use of calcium hypophosphite. Referring first to the effect of variation of the pH of the plating bath on the weight of nickel deposited in a given period of time when plating with calcium hypophosphite and calcium acetate as a buffer, the results of tests are shown by the curves 46, 48, 50 and 52 shown in Figs. 11 and 12 which record the weight of the nickel deposited in one hour with  $\text{Ni}^{++}/(\text{H}_2\text{PO}_2^-)$  ratios of 0.268, 0.402, 0.313 and 1.340, respectively.

The variation in the weight of the nickel deposited with change in the ratio of the nickel ions to hypophosphite ions, with different pH values, when the hypophosphite is derived from calcium hypophosphite in the presence of calcium acetate as a buffer is shown by tests, the results of which have been plotted to form the curves 54 and 56 in Fig. 13, where the abscissae indicate the ratios of nickel ions to hypophosphite ions and the ordinates show the weight of plating deposited in one hour in milligrams per square centimeter. The hypophosphite ion concentration was .224 mole/liter, the V/A ratio was 50  $\text{cm}^3/5 \text{ cm}^2$  and the acetate ion concentration was .120 mole/liter. The curve 54 shows the results when the pH of the bath had a value of 4.7 and the curve 56 shows the results when the pH was increased to 5.0. These results may be compared with those shown by Fig. 10 and also with those shown by Fig. 7, which represent the results of tests with hypophosphite ions derived from sodium hypophosphite.

## 10

With respect to the absolute quantity of buffer that has to be present in the plating bath, Reaction 3 above shows that, for every nickel ion reduced to the metal, two hydrogen ions are formed. In the absence of a buffer, the pH of the plating solution would therefore decrease rapidly below 4.0 with a corresponding loss of efficiency. The amount of buffer in the bath must therefore be sufficient to take care of the hydrogen ions that will be formed during the plating operation, i. e., corresponding to the maximum amount of nickel that can be reduced which, in turn is a function of the quantity of hypophosphite ion available.

The theoretical needed buffer concentration is the ion of an organic acid equivalent to two carboxyl groups for every nickel ion that can be deposited, for example, two moles of acetate for one mole of nickel. An excess of buffer, on the other hand, is objectionable, since it will lead to the formation of basic nickel salts. The amount of buffer which will give the best results may be readily determined by calculation.

To summarize some of the conclusions which may be drawn from the foregoing disclosure, it may be stated that, in order to obtain high rates of nickel plating by chemical means from the aqueous acid bath, without excessive formation of black precipitate (i. e., uncontrolled, random reduction of nickel) the following conditions should be fulfilled:

1. The ratio of nickel ions to hypophosphite ions in the bath should be between 0.25 and 0.60, depending upon the specific cation present.

2. The concentration of the bath in hypophosphite ions should be above 0.15 mole/liter and below 0.35 mole/liter.

3. The optimum initial pH values of the bath under the conditions indicated in the two next preceding paragraphs are in the range between 4.50 and 5.55. For instance, with sodium hypophosphite, there are two optimum initial pH values of 4.60 and 5.50, while when calcium hypophosphite is employed the optimum initial pH value is 5.0.

4. The buffer concentration in the bath should be equivalent to two carboxyl groups for every nickel ion that can be deposited.

5. The optimum ratio of solution volume of the bath to catalytic material area (V/A) is below 10.

It will be understood that the invention is not limited except as defined by the appended claims.

We claim:

1. The process of chemically plating with nickel a solid body essentially comprising an element selected from the group consisting of copper, silver, gold, aluminum, iron, cobalt, nickel, palladium and platinum, which comprises contacting said body with a bath consisting essentially of an aqueous solution of a nickel salt and a hypophosphite, wherein the ratio between nickel ions and hypophosphite ions in said bath expressed in molar concentrations is within the range 0.25 to 0.60, wherein the absolute concentration of hypophosphite ions in said bath expressed in mole/liter is within the range 0.15 to 0.35, and wherein the initial pH of said bath is within the approximate range 4.5 to 5.6.

2. The process set forth in claim 1, wherein said bath consists essentially of an aqueous solution of a nickel salt and a hypophosphite and a buffer in the form of a salt of an organic acid, and wherein the absolute concentration of said buffer in said bath is approximately two carboxyl groups for every nickel ion that can be deposited.

3. The process of chemically plating with nickel

## 11

a solid body essentially comprising an element selected from the group consisting of copper, silver, gold, aluminum, iron, cobalt, nickel, palladium and platinum, which comprises contacting said body with a bath consisting essentially of an aqueous solution of a nickel salt and a hypophosphite and a buffer in the form of an alkaline acetate, wherein the ratio between nickel ions and hypophosphite ions in said bath expressed in molar concentrations is within the 10 range 0.25 to 0.60, wherein the absolute concentrations of hypophosphite ions and acetate ions in said bath expressed in mole/liter are respectively approximately 0.225 and 0.120, and wherein the initial pH of said bath is within the approximate range 4.5 to 5.6.

4. The process set forth in claim 1, wherein the temperature of said bath is slightly below the boiling point thereof.

5. The process of chemically plating with nickel a solid body essentially comprising an element selected from the group consisting of copper, silver, gold, aluminum, iron, cobalt, nickel, palladium and platinum, which comprises immersing said body in a bath consisting essentially of an aqueous solution of a nickel salt and a hypophosphite, wherein the ratio between nickel ions and hypophosphite ions in said bath expressed in molar concentrations is within the range 0.25 to 0.60, wherein the absolute concentration of hypophosphite ions in said bath expressed in mole/liter is within the range 0.15 to 0.35, wherein the initial pH of said bath is within the approximate range 4.5 to 5.6, and wherein the ratio between the volume of said bath expressed in  $\text{cm}^3$  and the surface area of said body expressed in  $\text{cm}^2$  is not greater than 10.

6. A bath for the chemical plating of a catalytic material with nickel consisting essentially of an aqueous solution of a nickel salt and a hypophosphite, the ratio between nickel ions and hypophosphite ions in said bath expressed in molar concentrations being within the range 0.25 to 0.60, the absolute concentration of hypophosphite ions in said bath expressed in mole/liter being within the range 0.15 to 0.35, and the initial pH of said bath being in the approximate range 4.5 to 5.6.

7. A bath for the chemical plating of a catalytic material with nickel consisting essentially of an aqueous solution of a nickel salt and an alkaline hypophosphite and a buffer in the form of a salt of an organic acid, the ratio between nickel ions and hypophosphite ions in said bath expressed in molar concentrations being within the range 0.25 to 0.60, the absolute concentration of hypophosphite ions in said bath expressed in mole/liter being within the range 0.15 to 0.35, the absolute concentration of said buffer in said bath being approximately two carboxyl groups for every nickel ion that can be deposited, and the initial pH of said bath being in the approximate range 4.5 to 5.6.

8. A bath for the chemical plating of a catalytic material with nickel consisting essentially of an aqueous solution of a nickel salt and an alkali hypophosphite and a buffer in the form of a salt of an organic acid, the ratio between nickel ions and hypophosphite ions in said bath expressed in molar concentrations being within the range 0.25 to 0.60, the absolute concentration of hypophosphite ions in said bath expressed in mole/liter being within the range 0.15 to 0.35, the absolute concentration of said buffer in said bath being approximately two carboxyl groups for

70

## 12

every nickel ion that can be deposited, and the initial pH of said bath being in the approximate range 4.5 to 5.6.

9. A bath for the chemical plating of a catalytic material with nickel consisting essentially of an aqueous solution of a nickel salt and an alkali earth hypophosphite and a buffer in the form of a salt of an organic acid, the ratio between nickel ions and hypophosphite ions in said bath expressed in molar concentrations being within the range 0.25 to 0.60, the absolute concentration of hypophosphite ions in said bath expressed in mole/liter being within the range 0.15 to 0.35, the absolute concentration of said buffer in said bath being approximately two carboxyl groups for every nickel ion that can be deposited, and the initial pH of said bath being in the approximate range 4.5 to 5.6.

10. The process of chemically plating with nickel a solid body essentially comprising an element selected from the group consisting of copper, silver, gold, aluminum, iron, cobalt, nickel, palladium and platinum, which comprises contacting said body with a bath consisting essentially of an aqueous solution of a nickel salt and a hypophosphite, wherein the ratio between nickel ions and hypophosphite ions in said bath expressed in molar concentrations is within the range 0.25 to 0.60, wherein the absolute concentration of hypophosphite ions in said bath expressed in mole/liter is within the range 0.15 to 0.35, and maintaining the pH of said bath within the approximate range 4.5 to 5.6.

11. The process of chemically plating with nickel a solid body essentially comprising an element selected from the group consisting of copper, silver, gold, aluminum, iron, cobalt, nickel, palladium and platinum, which comprises contacting said body with a bath consisting essentially of an aqueous solution of a nickel salt and a hypophosphite, wherein the ratio between nickel ions and hypophosphite ions in said bath expressed in molar concentrations is within the range 0.25 to 0.60, wherein the absolute concentration of hypophosphite ions in said bath expressed in mole/liter is within the range 0.15 to 0.35, and periodically correcting the pH of said bath by the addition thereto of a soluble alkali to maintain a value within the approximate range 4.5 to 5.6.

12. The process of chemically plating with nickel a solid body essentially comprising an element selected from the group consisting of copper, silver, gold, aluminum, iron, cobalt, nickel, palladium and platinum, which comprises contacting said body with an aqueous bath consisting essentially of nickel ions, alkaline ions, hypophosphite ions and acetate ions, wherein the ratio between nickel ions and hypophosphite ions in said bath expressed in molar concentrations is within the range 0.25 to 0.60, wherein the absolute concentrations of hypophosphite ions and acetate ions in said bath expressed in mole/liter are respectively approximately 0.225 and 0.120, and wherein the initial pH of said bath is in the approximate range 4.5 to 5.6.

GREGOIRE GUTZEIT.  
ABRAHAM KRIEG.

References Cited in the file of this patent

UNITED STATES PATENTS

| Number    | Name    | Date          |
|-----------|---------|---------------|
| 1,207,218 | Roux    | Dec. 5, 1916  |
| 2,430,581 | Pessel  | Nov. 11, 1947 |
| 2,532,283 | Brenner | Dec. 5, 1950  |